

# UNITED STATES PATENT OFFICE.

TAKEJIRO SHIBATA AND EIICHIRO OE, OF KITA-KU, OSAKA, JAPAN.

## WATERPROOFING COMPOSITION AND PROCESS OF MAKING SAME.

1,380,428.

Specification of Letters Patent.

Patented June 7, 1921.

No Drawing.

Application filed May 6, 1918. Serial No. 232,684.

To all whom it may concern:

Be it known that we, TAKEJIRO SHIBATA and EIICHIRO OE, subjects of the Emperor of Japan, residing, respectively, at Kita-ku, 5 Osaka, Japan, have jointly invented certain new and useful improvements in Waterproofing Compositions and Processes of Making Same, of which the following is a specification.

10 Our invention relates to a waterproofing composition and the process of making same, and more particularly to a composition of this character especially adapted for use as a superficial coating for paper, for the purpose of protecting same from the action of moisture or fluid.

By means of the application of the composition of our invention to low grade paper stock, on either or both sides thereof, or as 20 a binder between superimposed plies of such stock, this stock is not only made impermeable by moisture, or fluids, but has imparted thereto properties similar to those of parchment paper. Furthermore, paper 25 stock treated with the composition of the invention is very much stronger than untreated paper stock of the same grade and weight.

The composition has little or no body, so 30 that its application to paper does not change the color of the paper, and in fact is imperceptible thereon except in so far as it imparts a parchment-like finish thereto. The composition as applied to the paper is odorless and has no injurious effects upon the paper, either as to its tissues, or its surface finish.

The invention consists primarily in a waterproofing composition embodying there- 40 in, in solution, acetate of aluminum and saponified vegetable oil; and in such other novel characteristics as result from the compounding of these ingredients in the manner hereinafter described and more particularly 45 pointed out in the claims hereto appended.

A waterproofing composition made in accordance with our invention, is composed of a saponified vegetable oil, emulsified in water, this emulsion having incorporated 50 therein aluminum acetate. In practice we have found that highly satisfactory results are obtained by using as the oil ingredient, a soap known commercially as "Marseilles soap" which analyzes substantially as follows:—Water approximately 22%, total fatty acids, including about 8% free fatty

acids, 68%, alkali about 8%, impurities 2%. The oil used in this soap is derived from the cocoanut or copra. This oil apparently reacts with the aluminum acetate producing insoluble salts, the excess of the oil being sufficient to impart flexibility to the paper, or other material, treated with the compound. 60

We believe that the insolubility of the compound after application to the paper, or other material, results from the chemical reaction between the said oil and the aluminum acetate and the small percentage of alkali in the soap is of secondary importance. 70

While in actual practice we have used saponified cocoanut oil, we believe that other vegetable oils such as cottonseed oil, could be advantageously used as a substitute therefor. 75

In the production of the compound, we employ the quantities of the several ingredients specified below and compound them as described. 80

In compounding substantially 16 gallons of the composition we first place approximately 1½ pounds (avoirdupois) of Marseilles soap in emulsion in 14 gallons of water, preferably distilled water, bringing 85 the mixture to substantially 212° F., or the boiling point thereof. When the mixture has been brought to the boiling point, we add approximately 2 gallons of distilled water and permit the temperature of the 90 mixture to fall below the boiling point without, however, cooling it materially.

To this emulsion, we add about 1 gallon of distilled water having in solution therein, approximately 4 ounces of aluminum acetate which has been thoroughly filtered while placing it in solution with the water. After the addition of the aluminum acetate, which is slowly added while the emulsion is still fairly hot, we permit the mixture to 100 cool slowly, while settling, thus affording ample time for the reaction between the oil and the aluminum acetate, which we find does not readily occur if the emulsion at the time of the addition of the aluminum acetate, is too cool, or if the mixture cools too rapidly after such addition. 105

If desired, coloring matter may be added to the compound but this is not essential to the invention. 110

When adding the aluminum acetate solution, this solution should be slowly mixed

with the emulsion, but thereafter the composition should not be agitated.

We used distilled water to avoid possibility of impurities which might interfere with uniformity in quality of the composition, although, we do not consider it absolutely essential to distil the water before placing the saponified oil in emulsion therein.

10 The composition thus produced is sufficiently viscous to be readily applied to sheets of paper with a brush, although, if desired, various mechanisms for spreading the composition upon the paper may be employed. The composition is sufficiently fluid, however, to permit it to be applied to paper by a dipping process if desired.

After application to paper, or other material, the composition should be allowed to dry under normal temperatures.

20 When dry, the composition forms a superficial, uniform coating upon the surface of the paper sufficiently bonded to the fiber to insure permanency of this surfacing. The 25 pores of the paper are well filled with the composition, and the flexibility of the composition prevents the formation of cracks therein through which water might seep in a manner to penetrate the fibers of the paper 30 and thus destroy its waterproof qualities. With some grades of paper, the composition will have an effect on the paper which causes the surface to be roughened similar to linen parchment papers. In all grades of 35 papers upon which we have used the composition, we find that the strength of the paper is materially increased.

We have also secured good results by 40 using the composition as a binder between separate plies of paper, not only more or less firmly uniting the plies, but providing an intermediate stratum having waterproof property, in the finished product in addition to the surface coating on either or both 45 sides thereof.

The proportions above specified may be varied without departing from the spirit and scope of the invention, no exactitude as to these proportions being requisite.

50 While we have specified the use of Marseilles soap in the production of the composition, other soaps might be used in lieu thereof, although, we have not secured highly satisfactory results with the use of 55 soaps made from animal fats.

It is not our intention to limit the invention to the precise characteristics of the composition or the steps of the process above specified, it being apparent that such may be 60 varied without departing from the spirit and scope of the invention.

Having described the invention what we claim as new and desire to have protected by Letters Patent is:—

1. A waterproofing composition the sole 65 active agents in which consist of the reaction products of acetate of aluminum and saponified vegetable oil.

2. A waterproofing composition the sole 70 active agents in which consist of the reaction products of acetate of aluminum and an emulsion of a cocoanut oil soap.

3. A waterproofing composition the sole 75 active agents in which consist of the reaction products of acetate of aluminum and an emulsion of an alkaline vegetable oil soap.

4. The herein described process of making a waterproofing composition consisting in emulsifying a saponified vegetable oil in 80 water, bringing the emulsion to its boiling point, adding a solution of acetate of aluminum while the emulsion is still heated, and slowly cooling the mixture.

5. The herein described process of making 85 a waterproofing composition consisting in emulsifying a cocoanut oil soap in water, raising the temperature of the emulsion to approximately 212° F. adding a solution of acetate of aluminum while the emulsion is 90 still heated, and slowly cooling the mixture.

6. The herein described process of making a waterproofing composition consisting in emulsifying an alkaline vegetable oil soap in water, raising the temperature of the 95 emulsion to approximately 212° F. adding a solution of acetate of aluminum while the emulsion is still heated, and slowly cooling the mixture.

7. The herein described process of making 100 a waterproofing composition consisting of compounding the following ingredients in substantially the following proportions and in substantially the following manner: Place 1 $\frac{1}{4}$  pounds avoirdupois of a vegetable oil 105 soap having an alkaline content of about 8% in 14 gallons of distilled water, raise the temperature to its boiling point (about 212° F.) add 1 gallon of distilled water containing in solution 4 ounces of acetate 110 of aluminum while the emulsion is still hot, and allow the mixture to cool slowly while settling.

In witness whereof, we hereunto affix our signatures, in the presence of two subscribing 115 witnesses, this 7th day of March, 1918.

TAKEJIRO SHIBATA.  
EIICHIRO OE.

Witnesses:

W. EBiharah,  
Ichiro Tuzaki.